# EUROPEAN PATENT SPECIFICATION

(11) **EP 0 205 423 B1**
(45) Date of publication and mention of the grant of the patent: **15.03.1989**
(21) Application number: 85900406.1
(22) Date of filing: 07.12.1984
(51) Int. Cl.: B05D 3/12, B05D 1/02, B05D 1/28, B05D 1/42, B05D 3/00, B05D 5/02, B05D 7/24

(54) **METHOD OF MAKING SIMULATED STONE AND WOOD**
VERFAHREN ZUR HERSTELLUNG VON KUNSTSTEIN ODER KUNSTHOLZ
PROCEDE DE FABRICATION DE PIERRE ET BOIS ARTIFICIEL

(43) Date of publication of application: 30.12.1986
(73) Proprietor: SCHIFFER, Henry, Boca Raton, FL 33435 (US)
(72) Inventor: SCHIFFER, Henry, Boca Raton, FL 33435 (US)
(74) Representative: Day, Jeremy John
(86) International application number: US8402032
(87) International publication number: WO8603433

(56) References cited:
- GB-A- 822 276
- US-A- 2 095 642
- US-A- 3 411 943
- US-A- 3 712 825
- US-A- 3 819 395
- US-A- 3 834 931
- US-A- 3 853 577
- US-A- 4 105 816
- US-A- 4 349 588

## Description

This invention relates to a method for making a simulated natural material surface on a wall, floor or roof according to the preamble of the only claim.

In the applicant's prior patent U.S. 4,349,588 a method is described for making a simulated brick or tile wall or floor using cement, water-based adhesive and optionally water-insoluble powdered pigment. The consecutive steps in that method consist of applying a mixture of the cement, water and water-based adhesive directly to a wall or floor, permitting partial setting, scoring selected indentations, permitting complete set, applying mortar into the indentations as a grout and then applying a clear water-resistant coating to the entire surface. Where color is desired a water insoluble powdered pigment is included in the initial mixture. In one variation, a clear coating is applied before applying the grout.

The method of the prior patent, while suitable for simulating brick or tile is not suitable for simulating stone, slate, wood or coral rock.

One object of the present invention is to provide a method for making simulated stone, slate, wood or coral rock.

The object is solved by the features as laid out in the characterizing portion of the only claim.

The method of this invention comprises first applying a coating of polyvinyl acetate latex emulsion to the existing surface to be covered and allowing the coating to dry. A mortar mixture made from a mixture of cement, sand, water and modified acrylic resin is then applied by trowel or with a spray nozzle from a hopper. The applied mortar mixture is permitted to partially set. Then, indentations in a selected design and/or desired surface texturing are made with appropriate tools to the partially set slurry. Excess material is then removed and the treated surface allowed to completely set and harden. After complete hardening, a first seal coating containing desired color or stain is applied. Alternately, a thin coat of the mortar mixture with shading color is applied, allowed to dry and then covered with a first clear seal coating. After the seal coating is dry any grout that is required can then be applied. This is followed by a final clear seal coating. The seal coatings in all cases are water-resistant.

The steps of the method of this invention are shown in the drawing which illustrates the steps of the process in making a simulated stone floor.

The following examples illustrate the invention:-

The references to I, II, III, IV, IVA, V and VI are to the drawing.

Example 1. A simulated stone floor is prepared by the following steps:

A 50% solid aqueous dispersion of polyvinyl acetate is applied to the surface to be covered and then allowed to dry. (1). After drying, a cement slurry is applied (II). Such a slurry typically consists of 5 gallons of water, 50 to 75 pounds of sand, 50 pounds, of Portland cement and 1-1/2 pounds of a modified acrylic resin emulsion having a high solids content. An example of such a resin emulsion is a commercial acrylic emulsion which has a solids content of 53%, viscosity of 300 centipoises, a specific gravity of 1.18 and a pH of 8.5. The slurry can be applied by either a trowel or a spraying apparatus. The depth of the slurry coating is in the range of 1/8 to one inch.

After the slurry coating is applied it is allowed to partially set, which typically takes two to three hours. When it is partially set, appropriate indentations according to a selected design and/or surface texturing are made with appropriate tools. (III). Thereafter, the excess materials are removed and the applied slurry allowed to completely harden. After this, a water-resistant seal coat containing the desired color or colors is applied. (IV). Where desired one seal coat of one color may be applied to a seal coat of another color before complete drying of the first seal coat, thus permitting blending, streaking and other similar desired effects. After the seal coats have completely dried required grout is applied. (V). The final step comprises applying a clear water-resistant seal coat to the entire surface. (VI).

Example 2. A simulated stone floor is prepared by the steps described in Example 1, except that instead of applying water-resistant seal coats containing color to the completely hardened surface, a thin coat of slurry containing shading color is applied, allowed to dry and then covered with a clear water-resistant seal coat. (IVA).

Example 3. Simulated wood is prepared by the same method as described in Example 1. The indentations are those which simulate the thin lines between wood planks. The texturing is much less than with simulated stone and the color in the first seal coat can be wood stain. Color can also be added to the wood grout.

## Claims

A method for making a simulated natural material surface on a wall, floor or roof comprising applying to the wall, floor or roof a mortar comprising a mixture of cement, water and water-based adhesive and allowing it to partially set; scoring indentations and/or surface texturing in a selected design in the partially set material and removing the excess material; allowing the mortar to completely set; applying a grout into the indentations and allowing it to set; and applying a clear water-resistant coating to the entire surface of the applied mixture, characterised in that the method is a method for making a simulated stone, slate, wood or coral rock surface; that prior to application of the mortar there is applied to the wall floor or roof a coating of a high solid aqueous emulsion of polyvinyl acetate, which coating is allowed to dry; that the mortar is an aqueous slurry of cement, sand and modified acrylic resin; and that prior to grouting either (a) a water-resistant seal coating containing desired colour is applied and allowed to dry or a thin coating of slurry containing shading colour is applied and allowed to dry and then a clear water resistant seal coating is applied.

## Patentansprüche

Verfahren Zur Herstellung einer künstlichen Naturmaterialoberfläche auf einer Wand, einem Boden oder Dach, umfassend das Aufbringen eines Mörtels, der eine Mischung aus Zement, Wasser und einem Haftmittel auf Wasserbasis aufweist, auf der Wand, dem Boden oder dem Dach und das teilweise Härtenlassen des Mörtels; die Einkerbung von Vertiefungen und/oder eine Oberflächentexturierung in einem ausgewählten Design auf dem teilweise gehärteten Material und das Entfernen des Überschüssigen Materials; das vollständige Härtenlassen des Mörtels; das Einbringen eines Vergußmaterials in die Vertiefungen und das Festwerdenlassen dieses Materials; und das Aufbringen einer klaren, wasserbeständigen Beschichtung auf die gesamte Oberfläche der aufgebrachten Mischung, dadurch gekennzeichnet, daß das Verfahren ein Verfahren zur Herstellung einer Kunststein-, Kunstschiefer-, Kunstholz-oder Kunstkorallensteinoberfläche ist; daß vor Aufbringen des Mörtels auf die Wand, den Boden oder das Dach eine Beschichtung einer hochfeststoffhaltigen wässerigen Emulsion aus Polyvinylacetat aufgebracht wird, welche Beschichtung man trocknen läßt; daß der Mörtel eine wässerige Aufschlämmung von Zement, Sand und modifiziertem Acrylharz ist; und daß vor der Vergußmaterialeinbringung entweder (a) eine wasserbeständige Dichtungsbeschichtung, die eine gewünschte Farbe enthält, aufgetragen wird und man diese trocknen läßt, oder eine dünne Beschichtung Tönungsfarbe enthaltender Aufschlämmung aufgetragen wird und man diese trocknen läßt und daß anschließend eine klare, wasserbeständige Dichtungsbeschichtung aufgebracht wird.

## Revendications

Procédé de fabrication d'une surface en matériau naturel simulé sur un mur, plancher ou toit, consistant à appliquer sur le mur, le plancher ou le toit un mortier comprenant un mélange de ciment, d'eau et de colle à base d'eau et à le laisser partiellement durcir; à réaliser des empreintes et/ou une surface fournissant une texture selon un dessin choisi sur le matériau partiellement durci et à enlever l'excès de matériau; à laisser le mortier durcir complètement; à appliquer un coulis dans les empreintes et à le laisser durcir; à appliquer un revêtement clair résistant à l'eau sur la surface totale du mélange appliqué, caractérisé en ce que le procédé est un procédé de fabrication d'une surface simulant la pierre, l'ardoise, le bois ou le corail; en ce qu'avant l'application du mortier on applique sur la paroi, le plancher ou le toit une émulsion aqueuse très ferme d'acétate de polyvinyle, lequel revêtement est laissé sécher; en ce que le mortier est une pâte épaisse aqueuse de ciment, sable et résine acrylique modifiée; et en ce qu'avant d'appliquer le coulis, soit l'on applique (a) un revêtement étanche résistant à l'eau contenant une couleur désirée et on le laisse sécher, soit on applique un revêtement mince de pâte contenant une couleur de nuançage et on le laisse sécher, puis un revêtement étanche clair résistant à l'eau est appliqué.
